

Oct. 25, 1927.

1,646,728

G. S. EVANS

## REFINING OF IRON

Filed June 7, 1926



**INVENTOR**  
*George S. Evans*

BY

BY  
Pennie, Davis, Harvey & Edmonds  
ATTORNEYS

## UNITED STATES PATENT OFFICE.

GEORGE S. EVANS, OF OAK PARK, ILLINOIS, ASSIGNOR TO THE MATHIESON ALKALI WORKS, OF NEW YORK, N. Y., A CORPORATION OF VIRGINIA.

## REFINING OF IRON.

Application filed June 7, 1926. Serial No. 114,157.

This invention relates to improvements in the refining of iron, and relates more particularly to improvements in the utilization of soda ash refining agents for this purpose. 5 Hitherto, in the utilization of soda ash in the refining of iron it has been considered impractical to use this refining agent except in an aggregated state, fused or briquetted or aggregated with other materials, due to the 10 loss and danger involved in dusting of the material where it was employed in the granular or pulverulent condition. This invention provides a method of handling refining agents such as soda ash and soda ash mixtures which makes it possible to employ these or similar materials in a granular or pulverulent condition without loss or danger.

In carrying out the process of the present invention, the refining operation proper is 20 effected primarily in a receptacle such as a bull ladle or mixing furnace in which a pool of the molten iron is subjected to the action of a fused refining slag containing the refining agent. This operation may, for example, be carried out as described in my prior 25 application filed April 10, 1925, Serial No. 22,047, a pool of iron being continuously maintained in the refining receptacle in contact with a slag bath continuously maintained 30 thereon, iron being supplied to and withdrawn from the pool during the operation without exhausting it and spent slag discharged and fresh refining agent added to the slag during the operation as required. 35 The present invention is also useful in connection with refining operations in which successive batches of iron are subjected to the action of a refining slag in such a bull ladle or mixing furnace or other refining receptacle. The present invention relates more 40 particularly to the operation by which the refining slag on the pool of iron in the refining receptacle is supplied thereto or by which fresh additions of refining agent are made 45 to such a slag on a pool of iron in the refining receptacle.

According to the present invention, the iron to be refined is passed as a molten stream 50 through an elongated passage way on its way to the refining receptacle and the granular or pulverulent refining agent is introduced into this passage way in contact with the stream of molten iron passing therethrough. The soda ash refining agent or 55 other refining material fusible at the tem-

perature of the molten iron is thereby sintered or melted to form an agglomerated mass or a fused slag which is permitted to pass with the stream of molten iron to the refining receptacle, and at the same time the pulverulent or granular refining material is confined to the passage way in which it is brought into contact with the molten iron until it is sintered or fused and it is not permitted to escape to the refining receptacle 60 until it has been agglomerated or melted and escape of the refining material into the surrounding atmosphere is thereby prevented.

The invention will be further described in 70 connection with the accompanying drawings which illustrate, in a diagrammatic and conventional manner, apparatus for carrying out the process of the invention. In the accompanying drawings:

Fig. 1 diagrammatically represents a section through the lower part of a cupola or melting furnace and of a bull ladle adapted to receive molten iron from the cupola or melting furnace,

Fig. 2 shows in a similar manner a modified arrangement of the cupola or melting furnace spout, and

Fig. 3 is a view similar to Fig. 2 showing a further modification.

The cupola or melting furnace illustrated is in general of the usual construction and operation and comprises a refractory lined shell 1 supported on legs 2, the furnace bottom 3, also refractory lined, being supported 90 on doors 4 held closed by support 5. A number of tuyères 6 are arranged opening into the furnace at some distance above the bottom and are connected to a common blast pipe 7. A slag spout 8 is also provided opening from the furnace a short distance below the tuyères. The cupola or melting furnace may be operated either with continuous tapping of the molten iron or with removal 95 of the molten iron from the cupola periodically with separation of the cupola slag in the cupola proper. In the first type of operation the cupola slag is caused to overflow through spout 9 being trapped from passing further by the dam 10. In the second type 100 of operation the cupola slag is periodically removed through spout 8. These types of furnace operation are well known and need not be described here.

In operation, the molten iron flows, either 110

intermittently or continuously according to the scheme of operation employed, from the cupola or melting furnace beneath the dam 10 through the passage way 20 formed by the cupola spout 11, the dams 10 and 12 and the refractory roof 13 to the refining receptacle 14, in this case a bull ladle with a bottom pouring spout 15 and a slag discharge spout 16. Arranged above the cupola spout 11 is a bin 17 from which refining material is fed into the passage way 20 by helical conveyer 18 of the usual type, the rate of supply of refining material to the passage way 20 being controlled by regulation of the speed of the conveyer. The bin 17 is kept supplied with the refining material from some suitable source through chute 19.

Granular or pulverulent soda ash or other refining material is supplied from the bin 17 to the passage way 20 while a stream of molten iron is flowing therethrough and is sintered or fused by heat from the molten iron to form an agglomerated mass or a fused slag which then passes with the stream of molten iron into the ladle 14. The dam 10 extending below the surface of the molten iron flowing through the cupola spout 11 effectively prevents the escape of any of the refining agent from the end of the passage way at which the molten iron enters. The dam 12 at the other end of the passage way is arranged to permit only a stream of sintered refining material or refining slag to escape with the molten iron into the refining receptacle. The refining material introduced into the passage way 20 is thus prevented from escaping until it is sintered or fused, and when it is sintered or fused it is permitted to discharge with the molten iron into the refining receptacle.

In the modified type of cupola spout illustrated in Fig. 2, instead of providing a dam, as shown at 12 in Fig. 1, to prevent the escape of unfused refining material at the end of the passage way from which the molten iron and fused refining material are discharged, the passage way 21 is prolonged sufficiently to insure that all of the refining material introduced at the end of the passage way at which the molten iron enters is sintered or fused before it can reach the other end of the passage way where the sintered or fused refining material is discharged with the molten iron.

In the modified type of cupola spout illustrated in Fig. 2, the passage way 22 is prolonged on both sides of the point of addition of refining material. This type of spout is more particularly adapted for use in connection with operations where the cupola slag is removed within the cupola. The molten iron, free from cupola slag in the cupola, flows as a stream through the passage way 22 at an intermediate point of which the refining material is added, the refining ma-

terial being sintered or fused before it can escape from the passage way, thus passing in sintered or fused condition with the molten iron to the refining receptacle.

If soda ash is used as a refining agent the amount employed per ton of iron may approximate 2 to 10 pounds per ton or maybe more than this. The batch type of operation usually requires a somewhat greater proportion of refining agent than the continuous type of operation if similar results are to be secured. In the batch type of operation, the refining material is added until a slag bath sufficient to treat the batch of iron is formed on the pool of molten iron in the refining receptacle and after sufficient time has passed to permit the refining operation to take place the spent slag is removed and the iron poured. In the continuous type of operation, where a pool of molten iron is maintained in the refining receptacle, it is advantageous to add fresh increments of refining material as additional molten iron is added to the receptacle if the cupola or melting furnace is tapped intermittently. Or if the cupola or melting furnace is tapped continuously, it is advantageous to supply refining material more or less continuously to maintain the refining slag on the pool of iron in the refining receptacle in a sufficient state of activity.

It will be apparent that this invention provides an improved method of operation which eliminates dusting or related difficulties where a refining agent such as soda ash is employed in a granular or pulverulent condition in the refining of iron. Loss and danger due to escape of the refining agent into the atmosphere are thus both avoided. Manual handling of the refining agent is also made unnecessary. While the invention has been described particularly in connection with the utilization of soda ash refining agents for this purpose, it will be apparent that it is also useful in connection with the utilization of other refining agents having similar properties. Another advantage of the present invention, which is particularly important in connection with operations in which the continuous type of refining operation is employed in conjunction with continuous tapping of the cupola or melting furnace, is that it makes it possible to supply the refining material progressively and substantially continuously so that the refining slag can be maintained at a more uniform activity and so that the refining operation can be more closely controlled.

The invention has further advantages in another aspect in that it provides for the addition of the refining agent in comparatively small increments to a likewise comparatively small stream of the molten iron to be refined. With refining agents which may contain or absorb moisture, the addition of

large batches of the refining agent to large batches of the molten iron may involve a danger of explosion due to flash vaporization of such moisture. In carrying out the present invention, the refining agent is added progressively to a flowing stream of the molten metal so that at no time is there any large amount either of the metal or of the refining agent present at the point of addition. Any danger of explosion is thus minimized, and any explosions that may result are of such minor magnitude that they can readily be confined, for example in the confined passage way in which the addition of refining agent is carried out. The progressive addition of the refining agent in carrying out this invention is also of advantage in making possible an improved proportioning between the refining agent and the molten iron.

I claim:

1. A process of refining iron which comprises flowing a stream of the iron in a molten state through an elongated passage way to a receptacle adapted to contain a pool of

the molten iron, introducing into the passage way in contact with the stream of molten iron a pulverulent refining agent fusible at the temperature of the molten iron, confining the pulverulent refining material so introduced to the passage way until sintered, and thereafter permitting the refining material to flow with the stream of molten iron to the said receptacle to form a refining slag on the pool of iron therein.

2. A process of refining iron which comprises flowing a stream of the iron in a molten state through an elongated passage way to a receptacle adapted to contain a pool of the molten iron, introducing into the passage way in contact with the stream of molten iron a pulverulent soda ash refining agent, confining the pulverulent refining agent so introduced to the passage way until sintered, and thereafter permitting the refining agent to flow with the stream of molten iron to the said receptacle to form a refining slag on the pool of iron therein.

In testimony whereof I affix my signature.

GEORGE S. EVANS.